

Oct. 11, 1955

J. F. KEGGIN

2,720,442

METHOD OF TREATING TOWS IN TUBES

Filed May 23, 1949



Inventor  
JAMES FARGHER KEGGIN

Cushman, Darby & Cushman  
Attorneys

1

2,720,442

**METHOD OF TREATING TOWS IN TUBES**

James F. Keggin, Seamill, Scotland, assignor to Imperial Chemical Industries Limited, a corporation of Great Britain

Application May 23, 1949, Serial No. 94,866

Claims priority, application Great Britain June 1, 1948

4 Claims. (Cl. 8—151.2)

The present invention relates to a method of treating a tow of filaments or threads in a limited space and is particularly concerned with a method of treating in non-tensioned condition a continuous tow of artificial filamentary products with a treating liquid having a specific gravity greater than the specific gravity of the tow.

It has been found to be difficult, e. g. to insolubilise in a satisfactory manner a continuous travelling tow of artificial filamentary products of vegetable seed globulins or phospho-proteins by allowing these products to fall into and accumulate or form folds in insolubilising solutions containing formaldehyde, sodium sulphate and sulphuric acid and of the kind which are of higher specific gravity than the said tow and are contained in a static tank of large but reasonable dimensions. The tow is found to form a compact floating mass difficult for the liquid to penetrate and the top of which is not in contact with the liquid, and to become entangled if a sufficient length is permitted to accumulate in the tank for it to receive the necessary time of treatment in the treating liquid.

Unsatisfactory results are also obtained if a tow of such filaments or threads is permitted to drop into and to form folds in the aforesaid liquids flowing through a static trough as tangling again results.

According to the present invention the method of treating in a non-tensioned condition a continuous tow of filamentary products with a treating-liquid having a specific gravity greater than the specific gravity of the tow comprises introducing a tow by means of a current of said treating-liquid through a tubular structure portion ending in a portion of preferably progressively increasing width leading to a tubular structure portion substantially wider than the narrowest part of the aforementioned tubular structure, arranging that the necessary length of the upper surface of the said wider tubular structure is at a lower level than the overflow level of the treating liquid and that the speed of the treating liquid through said tubular structures and the inclination upwards in the direction of flow of the said upper surface are such that the desired quantity of tow collects against the said upper surface and that the portion of the tow withdrawn from out of the treating liquid at the exit end of the broader tubular structure has remained in the treating liquid for the desired period of time.

The method of the present invention has been found particularly advantageous for the insolubilisation of continuous travelling tows of artificial filamentary products of protein with acidified concentrated saline solutions containing formaldehyde and of the kind which are of higher specific gravity than said tow.

The treating liquid and the tow pass through the narrower bore of the tubular structure at relatively high speed. The speed of the liquid here, which is controlled by the "head" or difference in level of the liquid at the entrance to the narrower tube and the exit of the wider tube or alternatively the pumping pressure, must be at least as great as that of the tow at this point. On enter-

2

ing the wider tube the tow folds irregularly and forms a loose column of fibre which moves slowly up the tube against the upper surface. This speed of travel in the wider tube is controlled to some extent by the speed of liquid flow in the wider tube, which depends on the relative bores of the narrower and wider tubes and the initial speed of the tow; and also on the inclination of the wider tube, for the fibre, being less dense than the liquid, tends to slide up the tube. Thus, the time of treatment of the fibre, which is the time taken to traverse the narrower and wider tubes, depends on the above factors controlling the speed of travel, and also on the length of the wider tube, or more accurately, on the length of the column of folded fibre allowed to accumulate in the wider tube before withdrawal. For a tow of given size and rate of delivery, the speed of liquid in the narrower tube, i. e. the "head," is adjusted to be somewhat greater than the tow speed. The bore size of the narrower tube is a matter of convenience. The size of the wider tube is then determined by the required time of treatment. It is possible to vary this time within very wide limits in the same apparatus, as the fibre may be drawn through both tubes with very little accumulation in a fraction of a minute, or may be allowed to accumulate in a longer column, the length of which is determined by the length of the wider tube, so that the time of passage may take many minutes.

Care has to be taken that the withdrawal of the tow from the treating liquid is in no way adversely affected by the treating liquid flowing out of the tubular structure of wider width and for this purpose it is desirable to provide said structure at the exit end with a perforated weir or an equivalent acting device.

Preferably the upper surface of said wider tubular structure is inclined at an angle lying between 5° and 30° to the horizontal.

The tubular structure portion having the narrow bore inlet is preferably of progressively increasing width, approaching or equal to the width of the tubular structure portion of wider width, in order to prevent excessive turbulence of the liquid flow and possible entanglement of the filaments forming the tow as it tends to rise in the treating liquid on entering the tubular structure of wider width.

The invention is illustrated by the following example in which parts are parts by weight except where otherwise stated and with reference to the diagrammatic drawing accompanying the application which is a front elevation of apparatus suitable for carrying out the method of the invention.

**Example**

A matured caustic soda solution of groundnut globulin prepared from a solution containing 20 parts peanut globulin, 1.25 parts sodium hydroxide, 1.0 part of sodium sulphite and 77.75 parts water is extruded into the coagulating bath containing 200 gms./l. sodium sulphate and 20 gms./l. sulphuric acid. The resulting tow of 15,000 filaments each of 3 to 4 denier is taken up on godets having a peripheral speed of 30 metres per minute and stretched by passing on to godets having a peripheral speed of 45 metres per minute.

The tow is then relaxed in a bath containing 300 gms./l. sodium chloride, 30 gms./l. sodium sulphate and not more than 3 gms./l. sulphuric acid at 20° C., removed from this bath by godets and passed into a setting bath containing 300 gms./l. sodium chloride, 30 gms./l. sodium sulphate, not more than 3 gms./l. sulphuric acid, and 5 gms./l. of formaldehyde, at 65° C. From this bath the tow 1 is removed by a godet 2 of peripheral speed 26 metres per minute and passes on to a godet 3 of peripheral speed 29 metres per minute, and then vertically downwards into the constant level feed cone 4, where it is

picked up by the hardening liquid which enters the feed cone through a pipe 5 and is then carried through the tube 6 and the glass cone 7 into the inclined tube 8. The tube 6 is of  $\frac{3}{4}$  inch diameter and the glass cone 7 is 4 inches in diameter at the open end. The composition of the hardening liquid is 111 gms./l. sodium chloride, 405 gms./l. sodium sulphate, 13 gms./l. formaldehyde and 303 gms./l. sulphuric acid, and it enters the tube 8 at 90° C. and overflows at 88° C. The speed of the liquid flow through tube 6 is controlled by the difference in levels of the liquid at the inlet cone 4 and the overflow at the exit end of the tube 8, which in this case is 4 inches. The tube 8 is of glass, 6 inches in diameter and 6 feet long, inclined so that the exit end is raised 14 inches above the inlet end. At the exit end of the tube 8 is attached a perforated lip 9 made of lead, which raises the level of the liquid in the tube 8 and allows it to flow away without giving rise to local regions of high speed flow. The speed of the tow at feed cone 4 is 29 metres per minute. On entering the inclined tube 8 through the funnel 7 the tow forms a loose column about 4 feet long against the upper surface of the tube 8 filling roughly about three quarters of the cross sectional area and is then removed at the exit end by a godet 10. The peripheral speed of this godet is adjusted to 21 metres per minute so that the time of passage through the tube 8 is constant and around 3 minutes, which is sufficient to insolubilise the protein fibre.

I claim:

1. A method of treating in a non-tensioned condition without tangling a continuous tow of artificial protein filaments which comprises introducing a tow of said filaments into the upper end of a longitudinally confined downwardly inclined treating zone of relatively small cross-sectional area, propelling said tow with a current of treating and carrying liquid having a specific gravity greater than the specific gravity of said tow through said first treating zone downwardly from the upper end thereof, said liquid completely filling said zone, moving said liquid together with the tow therein out of said first treating zone and directly therefrom into the lower end of a second longitudinally confined upwardly inclined treating zone of relatively large cross-sectional area in comparison with said first zone, said liquid completely

filling said second zone, carrying said tow through said second zone by moving said liquid in a non-turbulent condition through said second treating zone and withdrawing said tow from the upper end of said second treating zone.

2. A method as recited in claim 1 in which said downwardly directed narrow confined zone is substantially vertical and in which said upwardly inclined elongated confined zone has a cross-sectional area several times greater than the cross-sectional area of said narrow zone to insure an absence of turbulence in the major portion of said upwardly inclined zone.

3. A method as recited in claim 1 in which the treating liquor is an acidified concentrated saline solution containing formaldehyde.

4. A method as recited in claim 1 in which the time of treatment is varied by adjusting the velocity of the treating liquid and the angle of inclination of said upwardly inclined zone.

References Cited in the file of this patent

UNITED STATES PATENTS

|           |                    |                |
|-----------|--------------------|----------------|
| 430,817   | Anderson           | June 24, 1890  |
| 1,403,126 | Lyth               | Jan. 10, 1922  |
| 1,702,535 | Cole               | Feb. 19, 1929  |
| 1,825,478 | Rowley             | Sept. 29, 1931 |
| 1,871,100 | Walton et al.      | Aug. 9, 1932   |
| 1,913,601 | Leppin             | June 13, 1933  |
| 1,917,065 | Rusden             | July 4, 1933   |
| 2,131,409 | Nai                | Sept. 27, 1938 |
| 2,149,708 | Von-Recklinghausen | Mar. 7, 1939   |
| 2,156,090 | Hinnekens          | Apr. 25, 1939  |
| 2,267,117 | Mann               | Dec. 23, 1941  |
| 2,313,006 | Ufnowski           | Mar. 2, 1943   |
| 2,371,579 | Cole               | Mar. 13, 1945  |
| 2,377,434 | Lyem               | June 5, 1945   |
| 2,383,358 | Wormell            | Aug. 21, 1945  |
| 2,493,740 | Adams              | Jan. 10, 1950  |

FOREIGN PATENTS

|         |               |              |
|---------|---------------|--------------|
| 439,153 | France        | Apr. 1, 1912 |
| 13,626  | Great Britain | of 1889      |
| 467,257 | Great Britain | 1937         |